

# United States Patent

[11] 3,607,241

[72] Inventors **Gustaf F. Bolling**  
Dearborn;  
Jean Cisse, Dearborn Heights; Gerald S.  
Cole, Dearborn, all of, Mich.  
[21] Appl. No. **839,474**  
[22] Filed **July 7, 1969**  
[45] Patented **Sept. 21, 1971**  
[73] Assignee **Ford Motor Company**  
Dearborn, Mich.

[56] **References Cited**  
UNITED STATES PATENTS  
3,355,281 11/1967 Hansley et al. .... 75/138  
OTHER REFERENCES  
Orehoski, "Improved Crystal Structure in Cast Steel Ingots," Journal of Metals, May, 1969, Pages 41-48. Copy in  
Scientific Library of Patent Office.  
*Primary Examiner*—Richard O. Dean



PATENTED SEP 21 1971

3,607,241



FIG. 2



FIG. 3



FIG. 1

INVENTORS  
GUSTAF F. BOILING  
JEAN CISSE  
GERALD S. COLE  
BY John R. FAULKNER  
Thomas H. OSTER  
ATTORNEYS

## ALUMINUM-CASTING GRAIN REFINEMENT

## HISTORICALLY

This invention should be considered in view of the teachings of application Ser. No. 760,126, filed Sept. 13, 1968, and a more recent application Ser. No. 833,446, filed June 16, 1969. Both of these applications are filed in the names of G. F. Bolling and G. S. Cole and are assigned to the assignee of this invention.

These previously filed applications teach the control of grain structure particularly in castings which are approximate objects of revolution, either by slow rotation or very mild angular acceleration, about an axis preferably coincident with the axis of the casting. The speed of rotation or angular oscillation treated in all of these inventions is only of the order of 60 r.p.m. and is by no means to be confused with the much higher rates of rotation employed in conventional centrifugal castings.

The earlier applications mentioned above described in detail the casting of uninoculated INCO 713 turbine wheels. The only inoculation taught by these earlier applications is a minor inoculant coating of the mold as opposed to the present invention in which the inoculant is incorporated directly into metal whose solidification characteristics are to be controlled.

## THE INVENTION

This invention is related to the subject matter of both of the above-mentioned applications and particularly to the later filed application relating to the addition of an inoculant directly to the metal whose solidification characteristics are to be controlled. This later filed application teaches that the addition of an inoculant to a casting which is to be subject to slow rotation or oscillation during cooling directly reverses the results obtained with uninoculated castings. In the uninoculated castings steady-state rotation produces a columnar structure while angular acceleration or oscillation produces an equiaxed structure tending to be fine grained. In dealing with homologously inoculated castings, the diametrically opposite effect occurs with oscillations producing a columnar structure and rotation an equiaxed structure.

This invention is best depicted by typical metallographic studies which are shown in FIGS. 1 to 3.

FIG. 1 depicts the cross section of an argentiferous aluminum ingot containing as additional elements only 6.4 percent silver and cast normally.

FIG. 2 depicts the structure of an ingot consisting of an alu-

minum silver alloy also containing 6.4 percent silver. This alloy differs from that of FIG. 1 in that the silver was produced in situ by the addition of silver oxide to the melt. This initiated the typical thermit reaction and produced silver and freshly precipitated aluminum oxide. The aluminum oxide content was 1 percent.

FIG. 3 depicts the structure of an ingot containing 1.28 percent silver. This silver content of the alloy was also produced by the thermit reaction by the addition of silver oxide to the melt. This resulted in the concomitant production of 0.2 percent of freshly precipitated aluminum oxide.

The metallurgical structure depicted in FIG. 1 is that of gross columnar grains which one would normally anticipate upon the undisturbed cooling of an aluminum ingot in the uninoculated condition. The presence of 6.4 percent silver did not change the anticipated grain structure.

The structure depicted in FIG. 2 is an alloy of similar composition, but modified by the addition of the aluminum oxide in the freshly precipitated and very active form resulting from the oxidation of aluminum by added silver oxide which in turn is reduced to produce metallic silver. This addition considerably refined the structure and added a tendency to be partially equiaxed instead of completely columnar.

The structure shown in FIG. 3 shows the potent grain refining action of as little as 0.2 percent aluminum oxide which has been freshly precipitated in the melt. This melt was prepared by the addition to the melt of silver oxide sufficient to produce a silver content of 1.28 percent. The added silver oxide quickly reacted with the aluminum by the thermit reaction to produce metallic silver and a very active form of freshly precipitated aluminum oxide. In this particular ingot the normal grain refining action of the freshly precipitated aluminum oxide in the areas near the surface has been overpowered by the fact that this ingot was subject to angular accelerations during solidification. However, as the center of the ingot it approached the effect of these angular accelerations became negligible due to the small radius of gyration. In this inner area the very fine-grained structure produced by the freshly precipitated aluminum oxide in the undisturbed metal is very apparent.

We claim as our invention:

1. The process of refining the grain structure in an aluminum base casting comprising adding to the molten metal silver oxide, permitting the silver oxide to react with the molten metal to produce silver which alloys with the molten metal and freshly precipitated and very active aluminum oxide which acts as an effective aluminum grain-refining agent.